

## UNITED STATES PATENT OFFICE

2,495,918

POLY-N-VINYL LACTAM PHOTOGRAPHIC  
SILVER HALIDE EMULSIONSElmer Keiser Bolton, Wilmington, Del., assignor  
to E. I. du Pont de Nemours & Company, Wil-  
mington, Del., a corporation of DelawareNo Drawing. Application August 28, 1948,  
Serial No. 46,722

8 Claims. (Cl. 95—7)

1

This invention relates to photographic emulsions and emulsion layers composed of polymers of poly-N-vinyl lactams and to photographic elements containing such emulsion layers.

Many different materials have previously been used in photographic emulsions as binding agents for light-sensitive components. The most widely used material, gelatin, is well adapted to this use because it serves as a good protective colloid for silver halides in such emulsions and, when coated on a suitable support, these emulsions form films which are permeable to the aqueous solutions used to develop photographic images. Gelatin has a number of disadvantages, however, among which may be mentioned its high cost, lack of uniformity of one batch with another, susceptibility to bacterial attack, and its susceptibility to change in physical properties with changing humidity conditions.

It has now been found that useful photographic compositions can be made by incorporating light-sensitive material capable of forming a latent image, and especially silver halides, in a poly-N-vinyl lactam having an average molecular weight of about 10,000 to 500,000. This may be accomplished by dissolving the poly-N-vinyl lactam in water and admixing the light-sensitive silver halide therewith. After the light-sensitive material has been uniformly dispersed, the resulting colloidal dispersion may be further modified and coated on a support to form a light-sensitive layer.

In a practical mode of procedure, the poly-N-vinyl lactam, e. g., poly-N-vinyl caprolactam, is dissolved in water. Separate solutions are made by dissolving a soluble, ionizable halide, e. g., sodium, potassium, or ammonium chloride, bromide, or iodide, and by dissolving separately in water a soluble, ionizable silver salt, e. g., silver nitrate. The three solutions thus formed are mixed simultaneously to disperse colloidal light-sensitive silver halide in the polymer. The resulting emulsion can then be ripened, chilled, coagulated, and washed. Unwashed emulsions can be used but, in general, it is desirable to remove the excess soluble salts, preferably by dialysis. The precipitate can then be redispersed and the emulsion modified by the addition of more of the same type of poly-N-vinyl lactam, general emulsion sensitizers, anti-fogging agents, spectral sensitizing dyes, preservatives, hardeners, and/or color formers and coated on a temporary or permanent support or on a layer of such support.

After the light-sensitive poly-N-vinyl lactam solution is prepared for coating, it may be deposited in the same way that gelatin-silver halide

2

solutions are coated upon a suitable support, e. g., metal, paper, glass, or a transparent film such as a cellulose derivative, e. g., cellulose nitrate, cellulose acetate, or a superpolymer, e. g., polyvinyl chloride, polyethylene, nylon, etc., and dried. The resulting element can then be exposed and processed to positive or negative pictures in the same manner as ordinary gelatino-silver halide photographic elements.

10 The poly-N-vinyl lactams which have been found to be useful in the photographic emulsion layers of this invention can be made by adding a free radical producing catalyst, e. g., p-tertiary butyl peroxide,  $\alpha,\alpha'$ -azo-bis-isobutyronitrile, etc., 15 to N-vinyl lactams, e. g., N-vinyl caprolactam, and heating in the absence of oxygen until the polymer is formed. The useful poly-N-vinyl lactams have an average molecular weight of about 10,000 to 500,000 and are generally soluble 20 in water at 5° C. to 25° C. to the extent of 5%—20% or more. They can, however, be dissolved in water containing small amounts (10%—20%) of a water-soluble organic solvent, e. g., ethanol or methanol. The polymerization of N-vinyl caprolactam with  $\alpha,\alpha'$ -azo-bis-isobutyronitrile and related catalysts is disclosed and claimed in Hunt U. S. application Ser. No. 655,015, filed March 16, 1946, now abandoned, and continuation-in-part application Ser. No. 2,551, filed January 15, 1948, 25 now Patent No. 2,471,959.

30 The invention is further illustrated by the following examples in which parts are by weight. The photographic solutions and coatings were prepared in the absence of actinic light or radiations.

## Example I

40 A photographic emulsion containing poly-N-vinyl caprolactam having an average molecular weight of about 40,000 as the binder for silver halide was prepared as follows: Separate aqueous solutions containing the following constituents were made.

45 A  
AgNO<sub>3</sub> (3N) ----- cc. 29  
NH<sub>4</sub>OH (20%) ----- cc. 29  
Water ----- cc. 7

50 B  
NH<sub>4</sub>Br (3N) ----- cc. 31  
KI (0.5N) ----- cc. 2  
Water ----- cc. 32

55 C  
10% solution of poly-N-vinyl caprolactam in water ----- grams 100

These three solutions were mixed simultaneously by running streams of solutions A and B from separate containers into a common reaction vessel containing solution C with rapid agitation. The resulting light-sensitive silver halide suspension in the poly-N-vinyl caprolactam was dialyzed through a water-permeable cellophane (regenerated cellulose) membrane having a thickness of about 0.8 mil. until the conductivity had been reduced to 800 micromhos and coatings were made on raw stock paper coated with baryta gelatin. After drying, the photographic element was exposed by focusing on it the image of a transparency negative and developed by immersion at 20° C. in a standard p-methylaminophenol-hydroquinone developer having the following composition:

|                              | Parts |
|------------------------------|-------|
| p-Methylaminophenol sulfate  | 3.1   |
| Sodium sulfite (anhydrous)   | 45.0  |
| Hydroquinone                 | 12.0  |
| Sodium carbonate (anhydrous) | 67.5  |
| Potassium bromide            | 1.9   |
| Water to make                | 1,000 |

The developed picture was fixed by bathing in a 25% solution of sodium thiosulfate, freed from soluble salts by washing, and then dried. The resulting black and white picture had density gradations complementary to the object scene to which the element was exposed. The developed picture formed from the poly-N-vinyl caprolactam showed speed, contrast, and fog values comparable to that of commercial gelatino-silver halide emulsions used on enlarging papers. Prints on paper of this emulsion have a pleasing warmth of tone.

Similarly, a photographic emulsion can be prepared in which poly-N-vinyl caprolactam is used as a binder for light-sensitive silver halide and a color former. After exposing and processing in the usual manner with a color developer containing N-p-diethylaminoaniline, a photographic element bearing a colored photographic image can be obtained.

*Example II*

A photographic emulsion containing poly-N-vinyl-butyrolactam as the binder for silver halide was prepared as follows: Separate aqueous solutions containing the following components were made.

A

|                          |    |    |
|--------------------------|----|----|
| AgNO <sub>3</sub> (3N)   | cc | 35 |
| NH <sub>4</sub> OH (20%) | cc | 35 |

B

|                                                                                         |       |     |
|-----------------------------------------------------------------------------------------|-------|-----|
| NH <sub>4</sub> Br (3N)                                                                 | cc    | 37  |
| KI (0.5N)                                                                               | cc    | 6   |
| 10% soln. of poly-N-vinyl-butyrolactam<br>(average molecular weight of about<br>60,000) | grams | 120 |

Precipitation was made by adding solution A to B at 20° C. The precipitated silver halide particles were small (in the range of 0.05 to 0.2 micron diameter). The emulsion was washed by dialysis and coatings made according to the procedure described in Example I, with similar results.

The poly-N-vinyl-lactams which can be used in the process of this invention contain preferably from 4 to 6 carbon atoms in the inner amide or lactam ring and include poly-N-vinyl butyrolactam, poly-N-vinyl caprolactam and poly-N-vinyl

valerolactam. Mixtures of two or more of such lactams can be used. The poly-N-vinyl lactams should be capable of allowing the photographic processing solutions to penetrate sufficiently to act on the exposed and unexposed light-sensitive silver halide; at the same time, they should not dissolve in photographic processing solutions. To achieve this, they must have an average molecular weight of 10,000 to 500,000 or above.

The invention is not limited to the specific light-sensitive silver halides described in the above examples. Various other simple and mixed silver halides may be used as the light-sensitive materials of this invention. Mixtures of silver chlorides, bromides, and/or iodides can be made by adding mixtures of soluble salts of these halides in the same manner as described in Example I. Other useful soluble halides include potassium bromide, sodium iodide, sodium and potassium chlorides, etc.

The poly-N-vinyl lactams are useful not only as the binding agent for light-sensitive silver salts in radiation sensitive layers but may also be used as a water-permeable binder for other light-sensitive materials capable of forming a latent image such as diazonium compounds, ammonium bichromate, fulgides, N-monoarylhydroxylamines and their nitrones, etc. They may also be used as the binding agent of filter layers which may have dyes dispersed therethrough or antihalation layers which have antihalation dyes or pigments dispersed therethrough, and as binding agents for non-diffusing color formers which are placed adjacent to light-sensitive silver halide layers.

To the emulsions after formation and digestion can be added, either during the digestion stage or before, various types of sensitizing agents, e. g., sulfur sensitizers such as allyl thioureas, thiocyanates, or sodium thiosulfate. In addition, various types of optical sensitizing dyes which modify the spectral characteristics of the resulting emulsion can be added.

Various types of color formers or dye intermediates capable of forming quinoneimine, indophenol or azomethine dyes on color-forming development can be incorporated in the emulsions. Thus, the phenols, naphthols, pyrazolones, acylacetamides, hydrindene, N-homophthalimides, etc., particularly those of high molecular weight and which are immobile in gelatin emulsion layers can be used. Suitable color formers are described in United States Patents 2,108,602, 2,166,181, 2,178,612, 2,179,228, 2,179,238, 2,179,239, 2,182,815, 2,184,303, 2,186,849, 2,200,924, 2,283,276, and 2,328,652.

As compared with gelatin emulsions prepared under comparable conditions the poly-N-vinyl lactam emulsions contain smaller size particles of silver halide and, therefore, give emulsions that have less grain. The poly-N-vinyl caprolactam which is the preferred poly-N-vinyl lactam, has the unusual property of being soluble in water at temperatures below 30° C., but becoming practically insoluble as the temperature is raised to 30° C. and above. This unique property renders the silver halide emulsion layers useful in processing baths maintained at temperatures above 30° C. without reticulation. It is therefore superior to gelatin in this respect.

The light-sensitive film elements of the present invention can be used as a negative-taking stock, as positive print stock, or as reversal film, in the preparation of films for micro-copy, in X-ray films, in lithographic film, and as portrait materials. In fact, the film elements of this invention

tion can be used in systems in which elements based on gelatin or collodion have been used.

What is claimed is:

1. A photographic emulsion comprising light-sensitive silver halide grains dispersed in a poly-N-vinyl lactam having a molecular weight of about 10,000 to 500,000.

2. A photographic emulsion comprising light-sensitive silver halide grains dispersed in a poly-N-vinyl lactam having from 4 to 6 carbon atoms in the lactam ring and a molecular weight of about 10,000 to 500,000.

3. A photographic emulsion comprising light-sensitive silver halide grains dispersed in a poly-N-vinyl caprolactam having an average molecular weight of about 10,000 to 500,000.

4. A photographic element comprising a support bearing a photographic emulsion comprising light-sensitive silver halide grains dispersed in a poly-N-vinyl lactam having a molecular weight of about 10,000 to 500,000.

5. A photographic element comprising a support bearing a photographic emulsion comprising light-sensitive silver halide grains dispersed

in a poly-N-vinyl lactam having from 4 to 6 carbon atoms in the lactam ring and a molecular weight of about 10,000 to 500,000.

6. A photographic element comprising a support bearing a photographic emulsion comprising light-sensitive silver halide grains dispersed in a poly-N-vinyl caprolactam having an average molecular weight of about 10,000 to 500,000.

7. A photographic element comprising a transparent film support bearing a photographic emulsion comprising light-sensitive silver halide grains dispersed in a poly-N-vinyl lactam having from 4 to 6 carbon atoms in the lactam ring and a molecular weight of about 10,000 to 500,000.

8. A photographic element comprising a transparent film support bearing a photographic emulsion comprising light-sensitive silver halide grains dispersed in a poly-N-vinyl caprolactam having an average molecular weight of about 10,000 to 500,000.

ELMER KEISER BOLTON.

No references cited.